

S. G. HOWE.  
SAND BASE ROAD.  
APPLICATION FILED MAY 8, 1919.

1,355,833.

Patented Oct. 19, 1920.

Fig. 1



Fig. 2



Fig. 3



Inventor

Solon G. Howe

By *Whitney, Hall & Whitmore*

Attorneys

# UNITED STATES PATENT OFFICE.

SOLON G. HOWE, OF DETROIT, MICHIGAN.

## SAND-BASE ROAD.

1,355,833.

Specification of Letters Patent. Patented Oct. 19, 1920.

Application filed May 8, 1919. Serial No. 295,585.

To all whom it may concern:

Be it known that I, SOLON G. HOWE, a citizen of the United States of America, residing at Detroit, in the county of Wayne and State of Michigan, have invented certain new and useful Improvements in Sand-Base Roads, of which the following is a specification, reference being had therein to the accompanying drawings.

10 The invention relates to road construction and has particular reference to roads constructed over a sand base.

It is the object of the invention to dispense with costly foundations and at the same time to obtain a hard, durable and comparatively dustless surface. To this end the invention consists, first, in the method of construction, and, second, in the road, as hereinafter set forth.

20 In the drawings:

Figure 1 is a cross-section showing one form of construction;

Figs. 2 and 3 are similar views showing modified constructions.

25 Sand roads in dry weather are most unsatisfactory for travel. On the other hand, wet sand will pack so as to form a comparatively firm support where the area of bearing is not too restricted. Therefore a 30 comparatively thin surface layer of any good road material, such as crushed stone, if laid on wet sand will sustain the traffic, but when the sand dries the surface will soon break through. With my improvement a 35 permanent durable road can be built over a sand base by the use of a surfacing layer impregnated with a deliquescent salt, such for instance as calcium chlorid. This covering prevents the drying out of the sand 40 base and also operates to shed excess of rain-water so as to avoid washouts. When properly constructed and laid on a wet sand foundation such a road will remain in satisfactory condition for a long period of time, 45 while the expense of construction is only a fraction of that required for the building of a foundation.

In constructing my improved road the sand bed is first properly graded and provided with a curbing for protecting the edge portions from breaking away. This curbing may be cheaply constructed, as shown in Fig. 1, by driving stakes A to which are nailed wooden strips B of a width substan-

tially equal or slightly in excess of the depth 55 of the surface material. The road bed may be slightly rounded, if desired, and it may also be desirable to lay a line of drain tile at each edge, as indicated at C, the treated stone combination allowing a freer surface of 60 water to the drain tiles. Also it is preferable to increase the depth of the surface layer at the sides of the road, as indicated at D, where it extends downward to the drain tile C. The surfacing material may be made of 65 crushed stone, crushed cinders or other similar materials preferably reduced from one inch size down to dust and screened so as to give 34% ranging from dust to one-fourth 70 inch size and the remainder from one-fourth inch size to one inch. The dust and fine material will act as a carrier for the chemical and will fill the voids between the larger particles. The deliquescent salt is preferably in the proportion of 25 pounds of the 75 granulated salt to 6 gallons of water which is sufficient for 18 cubic feet of the prepared body materials. The materials are thoroughly mixed with the salt and are then spread over the graded base to a suitable depth, as for instance 4 inches, but before laying such surfacing material the base should be wet. When the road is completed it will have a comparatively hard but elastic surface which performs the double 80 function of distributing the load to the sand base and forming a blanket for retaining the moisture in the sand. In case of hard rains the excess of water will be shed from the round surface passing into the drains at 85 the sides and only sufficient water will percolate through the covering to maintain the moist condition of the sand.

In Fig. 2 I have shown a modification in which in place of a wood curbing a cement 95 curbing E and gutter E' are formed, said gutter being desirable where there are steep grades and a rapid flow of water. This figure also shows a line of central drain tile F at the center of the road with laterally 100 leading branches G to the sides. In Fig. 3 another modification is shown having a stone curb H and an adjacent ditch I filled with the surfacing material preferably carried down beneath the curbing; also a line of 105 drain tile J is arranged in said ditch. With all of these constructions as well as in other modifications that may be suggested the es-

sential characteristic is maintaining the sand base moist during dry weather and avoid washouts in wet weather.

What I claim as my invention is:

- 5 1. The method of constructing roads over a sand base, comprising properly grading the base and laying over the same while in moist condition a surfacing layer impregnated with a deliquescent salt.
- 10 2. The method of constructing roads over a sand base, comprising properly grading the base, placing a curbing at opposite sides thereof and laying over the same while in moist condition a layer of surfacing material impregnated with a deliquescent salt.
- 15 3. A road, comprising a moist sand base and a layer of surfacing material impregnated with a deliquescent salt.
4. A road, comprising a moist sand base, side curbing and a layer of surfacing material over said base between the curbs, said material being impregnated with a deliquescent salt. 20
5. A road, comprising a moist sand base, curbing at the opposite sides thereof, drainage means adjacent to said curbing and a layer of surfacing material between the curbs, said material being impregnated with a deliquescent salt. 25
6. A road, comprising a moist sand base and a layer of surfacing material composed of mixed fine and coarse road surfacing material impregnated with a deliquescent salt. 30

In testimony whereof I affix my signature.

SOLON G. HOWE.